

July 7, 1942.

O. SCHNECKO

2,289,049

ARTIFICIAL SAUSAGE CASING

Filed May 4, 1940



*Inventor.*  
Otto Schnecko

*By*  
*Hub, aff. Joslin*

HIS ATTORNEYS

## UNITED STATES PATENT OFFICE

2,289,049

## ARTIFICIAL SAUSAGE CASING

Otto Schnecko, Wiesbaden-Biebrich, Germany

Application May 4, 1940, Serial No. 333,369  
In Germany May 4, 1939

8 Claims. (Cl. 99—176)

The present invention relates to improvements in artificial sausage casings.

Various processes are already known for preparing tubular bodies, which may be used as artificial sausage casings, from papers coated with a film-forming substance or impregnated to a more or less large extent with the film-forming substance. The hitherto known products of this kind do, however, not fulfill all practical requirements. Moreover, the use of papers made of long fibers of quite a special genus of plants proved to be unsatisfactory.

Now I have found that a material which is particularly suitable for the manufacture of artificial sausage casings may be obtained by coating a fleece of artificial textile fibers, preferably a fleece of staple fibers of regenerated cellulose, with the film-forming substances. Fleeces of said fibers may be made in the usual manner by means of the devices known in the textile industry, for instance carding machines, whereas the hitherto used papers of long fibers are made, as is known, by a wet process. The fleeces of artificial textile fibers used according to the present invention are distinguished, in comparison with the papers consisting of long fibers, by their complete uniformity and the good felting property of the individual fibers. Moreover, particularly long fibers may be applied for the manufacture of the fleece. In consequence thereof tubular bodies which are made of impregnated fleeces of artificial fibers are of an extremely high strength and stability so that they fulfill all the requirements when they are used as artificial sausage casings.

According to the present invention, various kinds of film-forming substances, for instance albuminous substances, such as gelatin or casein, are used as impregnating agents; cellulose esters or cellulose ethers are also useful. Condensation products and polymerization products of various kinds, for instance those prepared from unsaturated halogen hydrocarbons, such as polyvinyl chloride, so-called "super-polyamides" and similar substances may likewise be used. Fleeces of artificial fibers coated with cellulose hydrate have particularly good properties. These cellulose hydrate coatings are produced in known manner, for instance with the aid of viscose or similar cellulose solutions.

I have furthermore found that the fleeces of artificial textile fibers which are very thin and fine and show only a slight inner coherence may best be further treated as follows: They are first treated, if necessary after having been cal-

endered, with only a very small quantity of the impregnating agent by applying it in the form of a solution to the fleece with the aid of squeezing rollers. After drying, the fleece thus reinforced is treated in the usual manner with the main portion of the impregnating agent. This treatment is known from the manufacture of tubular bodies consisting of impregnated paper. Owing to the preliminary impregnation the fibrous fleece has sufficient tensile strength so that it may be further treated while being unsupported. The finishing of the tubular body is very much accelerated thereby. Only a small portion of the entire impregnating agent to be used is preferably applied for the preliminary impregnation of the fibrous fleece.

It is particularly recommendable first to manufacture the casing from the reinforced fleece by folding the fleece, pasting together the overlapping edges and coating the tubular body thus obtained with the main portion of the impregnating agent. When operating according to this method particularly good casings having a very stable pasted seam are obtained. There is, for instance, obtained a tubular body useful as an artificial sausage casing by treating a fleece of artificial staple fiber material first with a quantity of the impregnating agent which amounts only to some percentages of the weight of the fleece, drying the fleece, shaping it to form a casing and then applying thereon a quantity of impregnating agent which is greater than the weight of the fleece and preferably amounts to a multiple of the weight of the fleece.

The tubular bodies thus pasted and impregnated may be finished in known manner by directly drying them or, if the impregnating agents used require it, subjecting them to a treatment with precipitating baths and cleansing baths and then drying them. If viscose is used as impregnating agent there is advantageously used for the precipitation, a bath known as "Müller"-bath and consisting of sodium sulphate and sulphuric acid. The tubular bodies are suitably dried in the inflated state. It may be advisable to treat the products with a softening agent before drying them.

The following example serves to illustrate a process of manufacturing tubular bodies according to the present invention. The process is illustrated by the accompanying drawing.

A fibrous fleece 1 is manufactured on a carding machine for artificial silk staple fiber of the usual construction (not illustrated in the drawing). The fleece consists of staple fibers of

regenerated cellulose and weighs about 20 grams per square meter (length of the staple fiber=3.5 cm.). When the fleece leaves the carding machine it is taken up by an endless conveying belt 2 which passes over the rollers 3 and 4. The fleece is then conducted to a pair of squeezing rollers consisting of rollers 5 and 6 which have been provided with a rubber coating. The lower roller 6 is partly immersed in a vessel 7 filled with viscose solution. It is suitable to use a viscose which contains 1.5 per cent of NaOH and 2 per cent of cellulose. With the aid of the squeezing rollers the fibrous fleece is impregnated with viscose. The pressure of the squeezing rollers is regulated in such a manner that the quantity of dry substance contained on the fleece after the impregnation amounts to about 4 grams per square meter of fleece. After having passed through the squeezing rollers the wet fleece impregnated with viscose is conducted over a large, driven drum 8, having a diameter of about 2 meters said drum being heated in the interior by steam. By means of an endless felted cloth 9 which passes over the rollers 10, 11, 12 and 13 the fleece is pressed onto the drum 8. In this manner the sized fibrous fleece is dried. The fleece then leaves the roller and by means of a conveying belt 14 which passes over rollers 15 and 16 it is brought to the place where it is further treated.

For the precipitation of the viscose and for a further purification as it is known in the manufacture of cellulose foils the weakly alkaline fleece of artificial silk staple fiber is passed through a number of treating baths in different tanks. The first of these tanks 17 is illustrated in the drawing. The fleece is conveyed in this case by means of driven rollers 18 which are situated in or above the tanks. For instance the following baths may be used: a precipitating bath containing about 5 per cent of sulfuric acid and 10-15 per cent of ammonium sulfate; a desulfurizing bath containing .5 per cent of sodium hydroxide or sodium sulfide and a bleaching bath (.2 per cent of active chlorine). Each bath is followed by a washing operation in a special tank. After having left the last bath the foil of artificial silk staple fiber thus treated is dried on a heated cylinder.

The reinforced staple fiber fleece obtained by the process described herein is cut into bands which are then pasted so as to form tubes and impregnated with the main portion of the viscose. For this purpose there is suitably used a viscose containing 5.8-6 per cent of sodium hydroxide and 7-7.5 per cent of cellulose, about three times the quantity of viscose, calculated upon the weight of the fleece being applied. The pasting of the sheet of artificial silk staple fiber to form a tube and the impregnation are carried out in the same manner as it is applied in the known

preparation of tubular bodies of impregnated paper. This known process is for instance described in U. S. Patents Nos. 2,105,273 and 2,144,900.

- 5 6. The fleece of artificial silk staple fiber may likewise be impregnated with a pasting agent other than viscose, for instance with a solution of gelatin or casein. If gelatin is used for pasting, it is applied in the form of an aqueous solution of 5 to 10 per cent strength, to which a small quantity of casein may suitably be added. The method of operating is the same as that described above, only the treatment in the precipitating bath and the subsequent purification are omitted.
- 10 I claim:
1. A sausage casing comprising a tubular body consisting of a fleece of staple fibers of regenerated cellulose and a coating upon the said tubular body which coating consists of a substance capable of forming a film.
2. A sausage casing comprising a tubular body consisting of a fleece of staple fibers of regenerated cellulose and a coating upon the said tubular body which coating consists of an organic substance capable of forming a film.
- 25 3. A sausage casing as claimed in claim 2 wherein the said coating consists of a substance capable of swelling in water.
- 30 4. A sausage casing comprising a tubular body consisting of a fleece of staple fibers of regenerated cellulose and a coating upon the said tubular body which coating consists of a film of regenerated cellulose.
- 35 5. A sausage casing comprising a tubular body consisting of a fleece of staple fibers of regenerated cellulose and a coating upon the said tubular body which coating consists of a film of an albuminous substance.
- 40 6. A process which comprises forming a tubular body from a fleece of staple fibers of regenerated cellulose, impregnating the said tubular body with a cellulose-solution and then after-treating the impregnated body so as to produce a coating of regenerated cellulose upon the said body.
- 45 7. A process as claimed in claim 6 wherein the said cellulose-solution is viscose.
- 50 8. A process which comprises applying to a fleece of regenerated cellulose staple fiber a quantity of viscose which amounts to only a fraction of the weight of the fleece, treating the fleece so as to precipitate the cellulose from the viscose solution, drying the fleece, forming a tubular body from the reinforced fleece applying a viscose solution in a quantity greater than the weight of the tubular body upon this body and aftertreating the material so as to produce a coating of regenerated cellulose on the said tubular body.

60 OTTO SCHNECKO.